# EUROPEAN PATENT SPECIFICATION

(11) **EP 0 219 927 B1**
(45) Date of publication and mention of the grant of the patent: **19.09.1990**
(21) Application number: 86305095.1
(22) Date of filing: 01.07.1986
(51) Int. Cl.: C10G 65/02, C10G 49/04

(54) **Process for preparing a very high quality lube base stock oil**
Herstellung hochqualitativer Grundschmieröle
Préparation d'huiles lubrifiantes de base de très haute qualité

(30) Priority: 10.07.1985 US 753478
(43) Date of publication of application: 29.04.1987
(73) Proprietor: MOBIL OIL CORPORATION, New York New York 10017 (US)
(72) Inventor: Bortz, Robert Walter, Woodbury Heights New Jersey 08097 (US); Graziani, Kenneth Richard, Woodbury New Jersey 08096 (US)
(74) Representative: Cooper, John Anthony

(56) References cited:
- GB-A- 1 566 233
- GB-A- 2 059 433

## Description

This invention relates to the manufacture of high grade viscous oil products from crude petroleum fractions. It is particularly directed to the manufacture of very high quality lube base stock oils from crude stocks of high wax content, commonly classified as "wax base" in contrast to "naphthenic base" crudes. The latter crudes are relatively lean in straight chain paraffins and yield viscous fractions which inherently possess low pour points.

Lube base stock oils are conventionally prepared by refining distillate fractions or the residuum prepared by vacuum distilling a suitable crude oil from which the lighter portion has been removed by distillation in an atmospheric tower. Thus, the charge to the vacuum tower is commonly referred to as an atmospheric resid or reduced crude, and the residuum from the vacuum tower is distinguished from the starting material by referring to it as the vacuum resid.

The vacuum distillate fractions are upgraded by a sequence of unit operations, the first of which is solvent extraction with a solvent selective for aromatic hydrocarbons. This step serves to remove aromatic hydrocarbons of low viscosity index and provides a raffinate of improved viscosity index and quality. Various processes have been used in this extraction stage employing solvents such as furfural, phenol, sulfur dioxide, and others. The vacuum resid, because it contains most of the asphaltenes of the crude oil, is conventionally treated to remove these asphalt-like constituents prior to solvent extraction to increase the viscosity index.

The raffinate from the solvent extraction step contains paraffins which adversely affect the pour point. Thus, the waxy raffinate, regardless of whether prepared from a distillate fraction or from a vacuum resid, must be dewaxed. Various dewaxing procedures have been used and the art has gone in the direction of treatment with a solvent such as methyl ethyl ketone (MEK)/toluene mixtures and/or catalytic dewaxing to remove the wax and provide a dewaxed oil. The dewaxed raffinate may then be finished by any of a number of sorption or catalytic processes to improve color and oxidation stability, e.g., clay percolation or hydrofinishing.

The quality of the lube base stock oil prepared by the sequence of operations outlined above depends on the particular crude chosen as well as the severity of treatment for each of the treatment stages. Additionally, the yield of a high quality lube base stock oil also depends on these factors and, as a rule, the higher the quality sought, the less the yield. In general, naphthenic crudes are favored because less loss is encountered, particularly in the dewaxing step. In many cases, however, waxy crudes are more readily available, and it would be desirable to provide a process for preparing very high quality lube base stock oils in good yields from such waxy crude oils.

In recent years techniques have become available for the catalytic dewaxing of petroleum stocks. U.S. Patent Re.No. 28,398 describes a process for catalytic dewaxing employing a catalyst comprising zeolite ZSM-5. Such a process combined with catalytic hydrofinishing is described in U.S. Patent No. 3,894,938.

U.S. Patent No. 4,437,975 describes a process for preparing a lube base stock oil from a vacuum resid by catalytically dewaxing the vacuum resid over a zeolite catalyst such as ZSM-5 and cascading the entire effluent, including hydrogen, into a hydrotreating reactor operated under relatively mild conditions, i.e., at a temperature from 260° to 357_{°}C (500_{°} to 675°F) and at a hydrogen partial pressure at the reactor inlet of 1034 to 10340 kPa.a (150 to 1500 psia). Under these conditions, the olefins present in the dewaxed feedstock are substantially hydrogenated thereby eliminating a principal source of oxidative and thermal instability. These hydrotreating conditions are not severe enough, however, to effect any appreciable reduction in the content of aromatic compounds and nitrogen- and sulfur-containing compounds the presence of which limits the use of the resulting oils to relatively undemanding service applications.

U.S. Patent No. 3,959,122 describes a process for producing a technical white oil having an ultraviolet absorptivity in the 280 to 289 millimicron region of less than 2.0 and having a viscosity in the range of 300 to 600 SUS (Saybolt Universal Seconds) at 38_{°}C (100_{°}F) in which a paraffinic distillate having a viscosity in the range of 400 to 600 SUS is hydrorefined at a temperature of 288_{°} to 316_{°}C (550_{°} to 600_{°}F), at a hydrogen partial pressure in the range of 5520 to 20685 kPa (600 to 3000 psi) and a total pressure in the range of 5520 to 41400 kPa g (800 to 6000 psig) in the presence of a sulfided nickel/molybdenum hydrogenation catalyst and at a liquid hourly space velocity (LHSV) of 0.1 to 1.0. Under these hydrorefining conditions, a significant reduction in aromatic, nitrogen and sulfur content occurs providing a very high quality oil which is suitable for demanding lubrication applications, e.g., as turbine oils.

British Published Patent Application No. 2059433A describes the preparation of lubricating oil basestocks by subjecting a petroleum vacuum distillate fraction or residue to a process including solvent extraction followed by mild catalystic hydrogenation at 310-450_{°}C over a sulfided hydrogenation catalyst containing oxides of molybdenum and nickel or cobalt followed by dewaxing.

This invention provides a process for preparing a very high quality lube base stock oil having excellent thermal and oxidation stability from a waxy crude oil. The process comprises:
(a) introducing an aromatic and nitrogen-and sulfur-containing feedstock selected from a dewaxed oil obtained from refining distillate fraction and having a 60 to 700 SUS at 38_{°}C (100_{°}F) and a dewaxed oil obtained from refining vacuum resid and having a 2300 to 2700 SUS at 38_{°}C (100_{°}F), and hydrogen, into a single stage hydrotreating reactor; and,
(b) subjecting the feedstock to hydrotreating in the reactor in the presence of a sulfided cobalt/molybdenum hydrotreating catalyst at an average reactor temperature from 316° to 357_{°}C at a hydrogen partial pressure from 13800 to 17240 kPa at the reactor outlet, an LHSV from 0.3 to 0.6 and a hydrogen circulation rate from 53.4 to 445 vol/vol (300 SCF (standard cubic feet) to 2500 SCF per barrel).

The use of a sulfided cobalt/molybdenum catalyst provides several advantages over a sulfided nickel/molybdenum catalyst as used in the hydrorefining process of U.S. Patent No. 3,959,122 referred to above. Thus, the greater stability of a cobalt/molybdenum catalyst compared to that of a nickel/molybdenum catalyst permits the former to be regenerated at a higher temperature and correspondingly shorter period of time than the latter thereby reducing reactor down-time and increasing productivity. In addition,the greater stability of the cobalt/molybdenum catalyst makes it more suitable for steam/air regeneration which is less expensive than the nitrogen/air regeneration methods more commonly employed with nickel/molybdenum catalysts. Moreover, cobalt/molybdenum is significantly easier to sulfide/presulfide, the form in which the catalyst must be used in the hydrotreating process herein. These advantages result in an overall superior hydrotreating operation compared to one employing a nickel/molybdenum catalyst.

Known unit processes are applied to distillate or vacuum resid fractions of waxy crude in particular sequence and within limits to prepare lube base stock oils used, for example, in hydraulic fluids, motor oils, turbine oils, marine oils and gear lubricants. The first step after preparation of a distillate fraction of suitable boiling range is extraction with a solvent which is selective for aromatic hydrocarbons, e.g., furfural, phenol, n-methylpyrrolidone, or others, to remove undesirable components of the fraction. With a vacuum resid fraction, it is required to propane deasphalt the resid prior to solvent extraction. In some instances, such as with a cylinder stock, solvent extraction of the deasphalted vacuum resid can be omitted. The raffinate from solvent extraction or propane deasphalting of vacuum resid is then dewaxed in a conventional manner, e.g., by treatment with a solvent such as MEK/toluene, propane or catalytically in the presence of hydrogen over a catalyst of an aluminosilicate zeolite having a silica to alumina ratio greater than 12 and a constraint index of 1 to 12 or by a combination of solvent and catalytic dewaxing as in U.S. Patent No. 3,755,138. The dewaxed oil is then hydrotreated in a single stage hydrotreating unit in the presence of sulfided cobalt/molybdenum catalyst operated under the foregoing specified conditions to provide a white oil possessing substantially improved color, demulsibility and oxidation stability and ideally suited for severe service applications such as turbine oils. The hydrotreated product is thereafter distilled, i.e., topped by distillation, to separate low boiling products of dewaxing in order to meet physical property specifications such as flash point and others. Conducting the unit processes at the conditions more fully specified hereinafter imparts high quality characteristics to the lube base stock oils and at the same time produces high yields of finished oils.

The wax base crudes (sometimes called "paraffin base") from which the charge stock is derived by distillation constitute a well recognized class of crude petroleums. Many scales have been devised for classification of crude, some of which are described in Chapter VII Evaluation of Oil Stocks of "Petroleum Refinery Engineering", W.L. Nelson, McGraw-Hill, 1941. A convenient scale identified by Nelson at page 69 involves determination of the cloud point of the Bureau of Mines "Key Fraction No. 2" which boils between 275_{°} and 300_{°}C (527_{°} and 572_{°}F) at 5330 kPa (40 mm) pressure. If the cloud point of this fraction is above -15_{°}C (5_{°}F), the crude is considered to be a wax base.

Known and conventional solvent extraction by counter current extraction with at least an equal volume (100 vol. %) of a selective solvent such a furfural is contemplated. It is preferred to use from 1.5 to 4.0 volumes of solvent per volume of oil. The furfural raffinate product is thereafter subjected to any one of several known and conventional solvent and/or catalytic dewaxing procedures.

Solvent dewaxing is a well known technique and needs no detailed description here. In general, the raffinate from the solvent refining unit is combined with a selective solvent and chilled to the appropriate temperature to crystallize the wax which is then separated therefrom. Representative examples of suitable solvents are (a) the aliphatic ketones having from 3 to 6 carbon atoms such as acetone, methyl ethyl ketone (MEK) and methyl isobutyl ketone (MIBK) and (b) propane, butane, and propylene as well as mixtures of the foregoing ketones and mixtures of the aforesaid ketones with aromatic compounds such as benzene and toluene. In addition, halogenated low molecular weight hydrocarbons such as the C₂-C₄ chlorinated hydrocarbons, e.g., dichloromethane and dichloroethane and mixtures thereof, can be used as solvents. Specific examples of suitable solvent mixtures are methyl ethyl ketone and methyl isobutyl ketone, methyl ethyl ketone and toluene, dichloromethane and dichloroethane and propylene and acetone. The raffinate is dewaxed by the selected solvent or solvent mixture which is adjusted to the composition of the charge stock to meet specifications for the particular lube base stock and the contemplated end-use, such being determined in accordance with well established practices.

In a preferred catalytic dewaxing procedure, the waxy raffinate from the solvent extraction operation is mixed with hydrogen and contacted at 260_{°} to 375_{°}C (500_{°} to 675°F) with a catalyst containing a zeolite ZSM-5 or other aluminosilicate zeolite having a silicate/alumina ratio above 12 and a constraint index of 1 to 12, with or without a hydrogenation component, and at an LHSV of 0.1 to 2.0 volumes of charge oil volume of catalyst per hour. The preferred space velocity is 0.5 to 1.0 LHSV. The catalytic dewaxing reaction produces olefins which would impair properties of the dewaxed oil product if retained. These are saturated by hydrogenation in the hydrotreating reactor. The saturation reaction is evidenced by the temperature rise in the first portion of the reactor, and confirmed by chemical analysis of the feed and hydrotreated product. By this means it is possible to prepare stable very high quality lube base stock oils having pour points even below - 54_{°}C (-65_{°}F).

In some instances it may be desirable to partially-dewax the charge stock to the catalytic dewaxing unit by conventional solvent dewaxing techniques as described above, say to a pour point of from -12_{°}C (10_{°}F) to about 10_{°}C (50_{°}F). The higher melting point waxes so removed are those of higher market value than the waxes removed in conventionally taking the product to a still lower pour point below -12_{°}C (10_{°}F).

The cracked (and hydrogenated) fragments from cracking wax molecules in the catalytic dewaxer will have adverse effects on the flash point of the dewaxed raffinate product and are therefore removed by distillation of the product to flash point specifications.

In the process of this invention, effluent from the solvent or catalytic dewaxing step (or sequential solvent/catalytic dewaxing operations) is introduced into a conventional fixed bed single stage hydrotreating reactor containing a sulfided cobalt/molybdenum catalyst on a support, e.g., one of alumina. Such catalysts are well known in the art and are commercially available. Shell's S 344 catalyst, a 1.6 mm (1/16 inch) pelletized extrudate of sulfided cobalt (2.4 wt. %) and molybdenum (9.8 wt. %) on alumina having a surface area of 190 m²/gm and a pore volume of 0.56 cc/gm has been found to provide entirely acceptable results.

The hydrotreating reactor is operated at an average reactor bed temperature from 316_{°} to 357_{°}C, a hydrogen partial pressure from 13800 to 17240 kPa.a, at the reactor outlet, an LHSV from 0.3 to 0.6, and a hydrogen circulation rate from 53.4 to 445 vol/vol (300 to 2500 SCF per barrel).

The effluent from the hydrotreating reactor is steam-stripped to remove the most volatile components and thereby meet flash point and other product specifications.

The following examples are illustrative of the process of this invention.

### EXAMPLE 1

An automotive grade furfural-extracted oil derived from a North Sea crude (Statfjord) which was dewaxed in a conventional manner employing a 65/35 toluene/MEK mixture was charged to a fixed bed single stage hydrotreating reactor of known construction loaded with Shell's S 344 sulfided cobalt/molybdenum on alumina hydrotreating catalyst.

The data for the conditions of the hydrotreating operation, the characteristics of the charge stock and the properties of the resulting hydrotreated oil in five separate cases are set forth in Table 1 as follows:

As these data show, in each case, the sulfur, nitrogen and aromatic content of the charge stock was substantially reduced providing very high quality lube base stock oils ("technical grade white oils") possessing much improved color and oxidation stability. The hydrotreated oils were entirely suitable for use as turbine oils.

### EXAMPLE 2

A high severity furfural-extracted distillate derived from a North Sea crude (Statfjord) which was subsequently dewaxed in a conventional manner with a 65/35 toluene/MEK mixture was subjected to hydrotreatment in the reactor and with the hydrotreating catalyst of Example 1 with the results (four cases) set forth in Table 2 as follows:

The lube base stock oil product in each of the four cases was a technical grade white oil of very high quality which is well suited for use as a turbine oil.

### EXAMPLE 3

This example illustrates the process of the present invention employing the reactor and catalyst of Example 1 but employing as the charge stock, a catalytically dewaxed solvent-extracted distillate of 200 SUS at 38_{°}C (100_{°}F) derived from a Mexican crude (Isthmus). The conditions of hydrotreatment, the properties of the charge stock and the properties of the hydrotreated oil (following steam stripping to remove volatiles) are set forth in Table 3 as follows:

The hydrotreated oil was of technical white oil grade and is well suited for use as a turbine oil.

## Claims

1. A process for obtaining a very high quality lube base stock which comprises:
(a) introducing an aromatic and nitrogen-and sulfur-containing feedstock selected from dewaxed oil obtained from refining distillate fractions and having a 60 to 700 SUS at 38_{°}C and a dewaxed oil obtained from refining vacuum resid and having a 2300 to 2700 SUS at 38_{°}C and hydrogen, into a single stage hydrotreating reactor; and,
(b) subjecting the feedstock to hydrotreating in said reactor in the presence of a sulfided cobalt/molybdenum hydrotreating catalyst at an average reactor temperature of from 316_{°} to 357_{°}C at a hydrogen partial pressure of from 13800 to 17240 kPa.a at the reactor outlet, an LHSV of from 0.3 to 0.6 and a hydrogen circulation rate of from 53.4 to 445 vol/vol to provide a very high quality lube base stock in which the aromatic, nitrogen and sulfur content is substantially reduced.

2. The process of claim 1 wherein the feedstock is a solvent dewaxed oil.

3. The process of claim 1 wherein the feedstock is a catalytically dewaxed oil.

4. The process of claim 1 wherein the feedstock is an oil which has been dewaxed by a combination of solvent dewaxing and catalytic dewaxing operations.

5. The process of claim 12 wherein the feedstock possesses an SUS at 38_{°}C in the range of 100 to 600.

6. The process of claim 1 in which volatiles are removed from the hydrotreated product of step (b).

## Patentansprüche

1. Verfahren zum Erhalt eines hochqualitativen Schmierölgrundmaterials, welches umfaßt:
(a) Einführung eines aromatischen und Stickstoff und Schwefel enthaltenden Ausgangsmaterials, das von entparaffiniertem ÖI ausgewählt wurde, das von der Raffination von Destillatfraktionen erhalten wurde und bei 38_{°}C eine Saybolt-Universal-Sekunde von 60 bis 700 aufweist, und von entparaffiniertem Öl, das aus der Raffination eines Vakuumrückstandes erhalten wurde und bei 38_{°}C eine Saybolt-Universal-Sekunde von 2300 bis 2700 aufweist, und von Wasserstoff in einen Einzelstufen-Hydrobehandlungsreaktor und
(b) Unterziehung des Ausgangsmaterials der Hydrobehandlung in dem Reaktor in Gegenwart eines sulfidierten Kobalt/Molybdän-Hydrobehandlungskatalysators bei einer durchschnittlichen Reaktortemperatur von 316 bis 357°C bei einem Wasserstoffpartialdruck von 13800 bis 17240 kPa.a am Reaktorauslaß, einer LHSV von 0,3 bis 0,6 und einer Zirkulationsmenge des Wasserstoffs von 53,4 bis 445 Vol.Nol., um ein hochqualitatives Schmierölgrundmaterial zu schaffen, bei dem der Aromaten-, Stickstoff- und Schwefelgehalt wesentlich reduziert ist.

2. Verfahren nach Anspruch 1, worin das Ausgangsmaterial ein mit Lösungsmittel entparaffiniertes Öl ist.

3. Verfahren nach Anspruch 1, worin das Ausgangsmaterial ein katalytisch entparaffiniertes Öl ist.

4. Verfahren nach Anspruch 1, worin das Ausgangsmaterial ein ÖI ist, das durch die Kombination von Lösungsmittetentparaffinierungs- und katalytischen Entparaffinierungsverfahren entparaffiniert wurde.

5. Verfahren nach Anspruch 12, worin das Ausgangsmaterial bei 38_{°}C eine Saybolt-Universal-Sekunde im Bereich von 100 bis 600 aufweist.

6. Verfahren nach Anspruch 1, worin die flüchtigen Bestandteile vom hydrobehandelten Produkt des Schrittes (b) entfernt sind.

## Revendications

1. Un procédé pour obtenir une huile lubrifiante de base de très haute qualité, caractérisé en ce qu'il comprend:
(a) l'introduction d'une charge d'alimentation contenant des produits aromatiques et de l'azote et du soufre, choisie parmi une huile déparaffinée obtenue par raffinage de fractions de distillat et ayant une viscosité de 60 à 700 SUS à 38_{°}C (100_{°}F) et une huile déparaffinée obtenue par raffinage d'un résidu sous vide et ayant une viscosité de 2300 à 2700 SUS à 38_{°}C (100_{°}F), et l'hydrogène, dans un réacteur d'hydrotraitement à étage unique; et
(b) la soumission de la charge à un hydrotraitement dans le réacteur en présence d'un catalyseur d'hydrotraitement au cobalt/molybdène sulfuré à une température moyenne du réacteur de 316_{°}C à 357_{°}C avec une pression partielle d'hydrogène de 13800 à 17240 kPa à la sortie du réacteur, une VSHL de 0,3 à 0,6 et un débit de circulation d'hydrogène de 53,4 à 445 vol/vol, pour fournir une huile lubrifiante de base de très haute qualité dans laquelle les teneurs en aromatiques, soufre et azote sont notablement réduites.

2. Un procédé suivant la revendication 1, caractérisé en ce que la charge d'alimentation est une huile déparaffinée par solvant.

3. Un procédé suivant la revendication 1, caractérisé en ce que la charge d'alimentation est une huile déparaffinée par voie catalytique.

4. Un procédé suivant la revendication 1, caractérisé en ce que la charge d'alimentation est une huile qui a été déparaffinée par une combinaison d'opérations de déparaffinage par solvant et de déparaffinage catalytique.

5. Un procédé suivant la revendication 1, caractérisé en ce que la charge d'alimentation présente une viscosité SUS à 38_{°}C de l'ordre de 100 à 600.

6. Un procédé suivant la revendication 1, caractérisé en ce que des volatils sont éliminés du produit hydrotraité de l'étape (b).
